

# United States Patent Office

2,696,472

Patented Dec. 7, 1954

1

2,696,472

## CORROSION INHIBITED LUBRICATING OIL

John M. Butler, Centerville, Ohio, assignor to Monsanto Chemical Company, St. Louis, Mo., a corporation of Delaware

**No Drawing. Application April 26, 1952,  
Serial No. 284,642**

**6 Claims. (Cl. 252—33.6)**

This invention relates to new lubricating oil compositions having a high degree of oxidation stability. More particularly the present invention relates to mineral lubricating oil compositions which have a materially decreased rate of corrosion in internal combustion engines, i. e. the gasoline and diesel engine and the like. This new improved lubricating oil comprises a mixture of a major amount of a hydrocarbon mineral lubricating oil and a minor amount of a member of the novel class of (tert-alkylmercapto)-zinc N,N-dialkyl dithiocarbamates or mixtures thereof.

The use of an improperly formulated lubricating oil can cause severe damage in the engine with which it is employed requiring extensive motor overhaul. This damage is primarily related to the corrosion of the bearing surfaces of the motor and can be attributed to a number of factors. Even high grade, carefully refined hydrocarbon lubricating oils are subject to oxidation and breakdown in the modern engine, wherein the conditions of agitation, high temperature and pressure, the presence of the fuel combustion products which get by the piston rings into the oil and metallic catalysts present in the system all contribute to altering the properties of the lubricating oil. The fuel combustion products which enter the lubricant are termed "blow-by gases" and generally contain metallic catalysts derived from the decomposition of anti-knock agents, etc. The alteration of the lubricating oil can also be accelerated by the bearing metal itself serving as a catalyst which metal surface is constantly reactivated by wiping. To meet this problem many oils contain additives which are generally called antioxidants or oxidation and bearing corrosion inhibitors.

and bearing corrosion inhibitors. Whereas the addition of efficient antioxidants are desirable in all lubricating oils they are particularly necessary in oils employed in engines containing bearing metals which are susceptible to corrosion, as for example, high-lead babbitts, cadmium alloys, copper-lead alloys, over-plated copper alloys, and the like, which types of bearing metals are employed in a large percentage of the engines currently in use.

It has now been found that the novel compounds having the illustrative formula:



wherein R represents a tert-alkyl radical containing from 8 to 16 carbon atoms and R' and R'' represent alkyl radicals containing up to 8 carbon atoms, have excellent properties as antioxidants in mineral lubricating oil compositions. The branched-chain alkyl radicals are specifically preferred for their oil-solubility characteristics.

The following (tert-alkylmercapto)-zinc N,N-dialkyl dithiocarbamates are illustrative of the novel antioxidants of this invention:

(Tert - dodecylmercapto) - zinc N,N - dibutyl dithiocarbamate,  
 (Tert-octylmercapto)-zinc N,N-dibutyl dithiocarbamate,  
 (Tert - dodecylmercapto) - zinc N,N-dimethyl dithiocarbamate,  
 (Tert - hexadecylmercapto) - zinc N,N - dioctyl dithiocarbamate,  
 (Tert-octylmercapto)-zinc N,N-dimethyl dithiocarbamate,  
 (Tert - decylmercapto) - zinc N,N - diisopropyl dithiocarbamate.

(tert-octyldimercapto)-zinc N-ethyl-N-methyl dithiocarbamate, and the like.

The exact means by which inhibitors decrease the potentially deleterious effects of a lubricating oil in an engine are not known. It has been suggested that inhibitors may function by decomposing the organic peroxides as formed to prevent a dangerous concentration built up of such compounds or may inactivate metallic catalysts present in the system and function, for example, as bearing metal passivators. Accordingly lubricating oil formulations cannot be readily evaluated by simple laboratory tests but require actual test in a motor under standard conditions defined to subject the formulation to conditions generally more severe than would be encountered in normal engine use. One such evaluation is known as the CRC Designation L-4-545 (CRC Handbook, 1946 Edition: Coordinating Research Council, Inc., pages 394-418) or the L-4 engine test, which test was designed to determine the oxidation and bearing-corrosion characteristics of lubricating oils and was employed to evaluate the formulations of the present invention.

The following example is illustrative of this invention. Lubricating oil compositions were prepared by mixing 0.5 and 1.0 parts by weight of (tert-dodecylmercapto)-zinc N,N-dibutyl dithiocarbamate with 100 parts by weight of a solvent refined Mid-Continent SAE 30 oil until a homogeneous solution was obtained. The above oil formulations were then evaluated with the standard L-4 engine test with the following results:

| Percent Antioxidant | Piston Varnish | Total Rating | Bearing weight loss in mg. |
|---------------------|----------------|--------------|----------------------------|
| 0.....              |                |              | >3,000                     |
| 0.5.....            | 8.9            | 91.4         | 564                        |
| 1.0.....            | 8.8            | 91.5         | 46                         |

It should be noted that tests were not completed using the straight mineral oil. Bearing weight losses of about 3000 mg. or more are meaningless for direct comparison with substantially lower values since practically all of the lead would be removed from the bearing and the corrosion rate would drop off rapidly. Thus the formulated oil compositions are substantially greater improvements than is indicated by the numerical data shown above.

60 is indicated by the numerical data shown above.  
The (tert-alkylmercapto)-zinc N,N-dialkyl dithiocarbamate antioxidants are employed in amounts of from about 0.1 to about 5 or more parts by weight and preferably from about 0.5 to about 2 parts by weight per 100 parts by weight of the lubricating oil.

65 parts by weight of the lubricating oil.

Other conventional motor oil additives can be used with the improved lubricating oil composition, as for example, other antioxidants, pour point depressants, viscosity index improvers, detergents, antifoam agents, rust-  
70 inhibiting dyes and the like.

70 The novel antioxidants disclosed herein and the process  
of producing them are described and claimed in my co-  
pending application, Serial No. 284,641, filed April 26,  
1952. The (tert-alkylmercapto)-zinc N,N-dialkyl thio-  
75 carbamate antioxidants are prepared by the reaction of  
(A) substantially equimolecular quantities of (1) a dialkyl  
amine, (2) carbon disulfide, and (3) an alkali metal hy-  
droxide in an aqueous medium; then adding thereto with  
agitation (B) a substantially equimolecular quantity of a  
80 zinc salt, wherein one anion is a water-solubilizing anion  
derived from a weak acid and the other anion is the tert-

alkylmercapto radical, dissolved in an inert water-immiscible solvent and continuing agitation for a sufficient time to effect substantially complete reaction. Then the solvent phase and the aqueous phase are allowed to separate and the aqueous phase removed and discarded. Thereafter the solvent phase is washed with water until substantially neutral and free from water-soluble salts. Then the solvent may be removed by distillation to recover the (tert-alkylmercapto)-zinc N,N-dialkyl dithiocarbamate.

I claim;

1. A lubricating oil composition comprising a major amount of a mineral lubricating oil and from about 0.1 to about 5 parts by weight per 100 parts by weight of the mineral lubricating oil of a (tert-alkylmercapto)-zinc N,N-dialkyl dithiocarbamate antioxidant having the formula:



wherein R represents a tert-alkyl radical containing from 8 to 16 carbon atoms and R' and R'' represent alkyl radicals containing up to 8 carbon atoms.

2. The lubricating oil composition of claim 1 wherein the antioxidant is (tert-dodecylmercapto)-zinc N,N-diethyl dithiocarbamate.
  3. The lubricating oil composition of claim 1 wherein the antioxidant is (tert-octylmercapto)-zinc N,N-dipentyl dithiocarbamate.
  4. The lubricating oil composition of claim 1 wherein the antioxidant is (tert-hexadecylmercapto)-zinc N,N-dimethyl dithiocarbamate.
  - 10 5. The lubricating oil composition of claim 1 wherein the antioxidant is (tert-hexadecylmercapto)-zinc N,N-diethyl dithiocarbamate.
  - 15 6. The lubricating oil composition of claim 1 wherein the antioxidant is (tert-dodecylmercapto)-zinc N,N-diethyl dithiocarbamate.

**References Cited in the file of this patent**

UNITED STATES PATENTS

20 Number Name Date  
2,400,106 Dension et al. May 14, 1946